

## UNITED STATES PATENT OFFICE.

PHILIPPE DE CLAMECY, OF BOSTON, MASSACHUSETTS, ASSIGNOR TO B. E. STURTEVANT COMPANY, OF HYDE PARK, MASSACHUSETTS, A CORPORATION OF MASSACHUSETTS.

## STEEL AND IRON ALLOY.

No Drawing.

Application filed October 6, 1919. Serial No. 328,685.

*To all whom it may concern:*

Be it known that I, PHILIPPE DE CLAMECY, a citizen of the United States, residing at Boston, in the county of Suffolk and State 5 of Massachusetts, have invented certain new and useful Improvements in Steel and Iron Alloys; and I do hereby declare the following to be a full, clear, and exact description of the invention, such as will enable others 10 skilled in the art to which it appertains to make and use the same.

The invention relates to steel and iron alloys.

The object of the invention is to provide 15 steel and iron alloys which not only have the usual characteristics adapting them to the various commercial uses for which they are intended but also are non-corrosive and non-rusting under conditions which render 20 the use of the usual commercial irons and steels impracticable or which result in their rapid deterioration or destruction.

I have found that by the addition to commercial pig irons or steels of small percentages of cobalt, nickel, chromium and silicon, 25 alloys may be produced which are not acted on or attacked by gaseous fumes or vapors of sulphur or solutions of sulphuric acid and are not oxidized when subjected to the 30 usual oxidizing atmospheres. The proportions which I have found to give highly satisfactory results are 2½% cobalt, 2% nickel, 1½% chromium and 1½% silicon. These proportions may be varied somewhat 35 but should not be increased sufficiently to render the resulting alloy unfit for commercial use or reduced sufficiently to seriously impare its non-corroding and non-rusting qualities. For instance, I have found that

40 an increase of the cobalt and chromium above 6% and of the nickel and silicon above 7½% and 3% respectively renders the resulting alloy too brittle for commercial use, although it is still non-corrosive and its 45 rust resisting qualities are increased. On the other hand the reduction in the percentages to cobalt 1½%, nickel ¾%, chromium

½% and silicon ½% destroys the acid resisting qualities of the alloy and renders it easily rusted. I have also found that in no 50 case should the alloy contain more than 3% carbon.

In case the iron or steel to be treated already includes any of the elements referred to, the percentage of such element present 55 should of course be allowed for in the production of the alloy. The alloys may be produced by adding the elements referred to to pig iron or steel already manufactured or may be incorporated in the original manu- 60 facture.

By the inclusion of the elements referred to in approximately the proportions mentioned, iron and steel may be produced which is not materially affected by the action 65 of the corrosive fumes and vapors of sulphur and of any solution of sulphuric acid and by the oxidizing and rusting action of moisture and air while retaining the tensile strength, malleability and other characteristics which render it particularly adapted 70 for the commercial use for which it may be intended. These alloys may therefore be used with particular advantage in the manufacture of apparatus, such for instance 75 as economizers and blowers, for use under conditions in which it handles or is subjected to the action of corrosive or oxidizing gases, fumes, or vapors. This alloy also has the further advantage that it may be easily 80 annealed to contain not more than .9% carbon and then allowed to quench in the atmosphere thereby giving a good temper to the annealed alloy.

What is claimed is:

1. An alloy of iron or steel, containing over 1½% and less than 6% of cobalt, over ½% and less than 6% of chromium, over ¾% and less than 7½% of nickel, and over ½% and less than 3% of silicon.

2. An alloy of iron or steel, containing approximately 2½% cobalt, 2% nickel, 1½% chromium, and 1½% silicon.

PHILIPPE DE CLAMECY.